

1

3,429,651

**REACTIVE DRESSINGS INTENDED TO RENDER  
CELLULOSE FABRICS UNCREASABLE**

Pierre Talet, Alfortville, and Louis Gandon, Trosly-Breuil,  
France, assignors to Nobel-Bozel, Paris, France, a 5  
joint-stock company of France  
No Drawing. Filed May 11, 1965, Ser. No. 454,990  
Claims priority, application France, May 13, 1964,  
974,388

U.S. Cl. 8—116.3  
Int. Cl. D06m 13/38

11 Claims

10

**ABSTRACT OF THE DISCLOSURE**

A process is disclosed for treating cellulose fabrics with cyclic urea-formol resins to provide "wash and wear" fabrics which are resistant to chlorine degradation. This is accomplished by utilizing with the dressing resin in a catalyst of glyoxylic acid.

The present invention relates to the treatment of cellulose fabrics with known resins, modified however by glyoxylic acid, and in particular to an improved method for rendering such fabrics still more uncreasable and to treatment with chlorine, especially washing followed by treatment with chlorine, especially washing with the so-called "Javel water" (an aqueous solution of sodium hypochlorite and sodium chloride).

It has already been proposed to render cellulose fabrics, particularly cotton, uncreasable by applying to them methyloated derivatives of ethylene-urea, mono-ureine of glyoxal, that is to say of imidazolidinone-2, and glycoluryl, and then causing the reaction of these different reactive dressings by the methyloated groups with the cellulose in order to etherify this latter.

These types of dressings belong to the group of the methyloated derivatives which are difficult to condense on themselves, but which react readily on the hydroxyl groups of cellulose. They result in fabrics having good "wash and wear" characteristics, the value of which can only be determined by visual comparison of the fabrics after washing, with reference to types such as those proposed by the A.A.T.C.C. In fact, these qualities give the natural fibres the ability to retain their shape during washing, rapidity of drying, uncreasing after creasing, strength in the dry and wet states and great resistance to washing, while giving properties of good tensile strength, good resistance to tearing and to abrasion.

The above-mentioned products belong to the group of cyclic-formol ureas and do actually give these general effects. Unfortunately, in countries in which household linen and underwear are treated with Javel water after soaping, the resistance of the dressings to chlorine is the basis of their choice. It is known that apart from the methyloltriazinones, which although they absorb chlorine do not cause any appreciable attack during the ironing of the dressed cellulose, the above-mentioned resins give rise to a very considerable degradation of the fabrics during the course of these operations.

A considerable amount of work has been carried out in laboratories in order to determine the mechanism of the action of chlorine and that of the attack of cellulose during ironing. The factors have been discovered which influence the stability to chlorine and the evolution of the latter during the course of successive washings.

The fixation of the cellulose with the  $\text{CH}_2\text{OH}$  groups would be effected by the formation of co-valent bonds with the elimination of water. Furthermore, the hypochlorous ion can be fixed like chlorine on the nitrogen of the methylolamides when the latter processes hydrogen

2

atoms directly associated with nitrogen, to form chloramides.

The chloramides formed are stable during washing and can only be destroyed by the action of a de-chlorinating product such as bisulphite, hydrogen peroxide, perborate.

The formation of these chloramides is indicated by the appearance of a slight odour of chlorine and a yellowish colour. They decompose under heat during ironing for example, liberating hydrochloric acid and nascent oxygen. The cellulose is degraded simultaneously by the hydrochloric acid and the nascent oxygen. This rapid degradation while hot can also occur, but very slowly, by the action of light and moisture.

In the case of methyloated cyclic ureas which no longer comprise CO—NH groups capable of fixing chlorine following the reaction:



there is however observed a poor resistance to chlorine of the fabrics treated. This must be attributed to the fact that a certain percentage of  $\text{CH}_2\text{OH}$  groups have remained free and become hydrolysed so as to re-form the CO—NH groups, and these, when re-introduced on to the fibre, render it sensitive to chlorine.

Catalysts such as tartaric, lactic, oxalic and glycolic acids, while they are suitable for uncreasable dressings containing dimethylol-urea, are not suitable for the methyloated cyclic ureas such as dimethylol-ethylene-urea.

It could therefore not be foreseen that glyoxylic acid should prove suitable for acting as a catalyst with the cyclic ureas.

Now, according to the present invention, the applicants have found that glyoxylic acid is perfectly suitable as a catalyst with certain cyclic ureas. Furthermore, even when applied alone, glyoxylic acid has an action as an agent intended to give fabrics good uncreasability, which fact has not been observed up to the present time.

The invention is characterized by the fact that glyoxylic acid, by its nature as an acidic catalyst and by its aldehyde function which enables it to become fixed on cellulose by causing a reticulation between the chains, gives certain methyloated cyclic ureas the possibility of supplying highly uncreasable fabrics which are resistant to the action of chlorine.

Without departing from the scope of the invention, it is possible to add to solutions containing glyoxylic acid and the methyloated derivative, a more or less considerable quantity of metallic salts currently employed as condensation catalysts, such as: hexahydrated magnesium chloride, hexahydrated zinc nitrate, etc.

Other agents employed in the industry of uncreasable fabrics, such as softeners, high vinyl, acrylic, etc., polymers, may be present in the impregnating solution or may be added subsequently.

In order to obtain at the same time uncreasability and resistance to chlorine, it is essential that the ratio of the methyloated derivative to glyoxylic acid is such that the glyoxylic acid present exercises a sufficient action on the condensation of the methyloated groups in order that, at the end of the treatment, the latter have wholly entered into reaction.

In order to facilitate this complete reaction of the methylols which is essential in order that the resistance to chlorine may persist after several washings, the function of the glyoxylic acid as a condensation catalyst may be completed by other inorganic or organic catalysts.

The cyclic methyloated derivatives suitable for the method of the invention are for example those which are particularly described in the present applicants' French Patent No. 1,351,590 of Dec. 28, 1962.

Dimethylol dihydroxy-ethylene-urea also gives very improved performances by catalysis with glyoxylic acid.

The aqueous solutions are employed in variable concentrations, the proportion of glyoxylic acid with respect to the dressing being in percentages ranging from 10% to 100%, and preferably between 33% and 50%.

The amount of absorption by the wet fabric is regulated so that the increase in weight is comprised between 2 and 20% or more, the optimum proportion being in general between 5 and 12%. The proportion of glyoxylic acid based on the anhydrous product may vary from 1% to 100% by weight with respect to the dry methyloated derivative.

In the tests which follow, given by way of illustration and not in any way restricting the present invention, the parts and percentages are indicated by weight.

The tests of which the results are given in the examples were carried out on the fabric treated which was kept at 20° C. and a relative humidity of 65%. The tensile strength given in kgs., forms the subject of the French AFNOR specification G-07-001-44.

The resistance to chlorine (Scorch Test) is measured in accordance with the Tentative Test Method 92-1958-t, adopted in 1961 by the A.A.T.C.C. (American Association of Textile Chemists and Colorists).

The flattening angle, after a wrong fold in the dry state,

following the method adopted by Monsanto, by reference to the sample comprised in the Monsanto Three-Dimensional Standard, Tentative Test Method kit, following the proposal of the A.A.T.C.C.

#### EXAMPLE 1

Utilizing a condensate of cyclic methyloated urea modified by acryl-amide prepared under the conditions defined in the French patent referred to above, this is diluted until a solution is obtained having 15 grams of dry product per litre. Impregnations were made by padding a cotton fabric of the reinforced cretonne type, bleached 32-32, 50-50, of 132 grams per square metre.

Wringing rates of the order of 90% are employed. All the sample pieces are placed on a frame and dried at 90° C. for 10 minutes before being condensed for 5 minutes at 150° C. in a ventilated oven.

The results are given in Table I below. By way of comparison, the results obtained with the usual catalysts, magnesium chloride, zinc nitrate, are also shown.

In this table, and also in all the other tables which are given below, the values shown in parentheses represent the sum of the values indicated for "Warp" (Wp) on the one hand and "Weft" (Wt) on the other.

TABLE I

| Test No. | Bath formula and working conditions                                                                                                                | Dynamo Strength (kg.) Wp/Wt | Uncreasability |               | W & W Monsanto test |        | Whiteness (as it is) | Scorch test A.A.T.C.C., percent |        |
|----------|----------------------------------------------------------------------------------------------------------------------------------------------------|-----------------------------|----------------|---------------|---------------------|--------|----------------------|---------------------------------|--------|
|          |                                                                                                                                                    |                             | As it is Wp/Wt | 2 wash Wp/Wt  | 2 wash              | 5 wash |                      | As it is                        | 5 wash |
| 354..... | Methyloated derivative (dry state), 15 g.; MgCl <sub>2</sub> ·6H <sub>2</sub> O, 6.65. Drying at 90° C. for 10 min. Condens. at 150° C. for 5 min. | 29.8/30.1 (59.9)            | 133/132 (265)  | 139/143 (282) | (1)                 | (1)    | 81                   | 33                              | -----  |
| 294..... | Methyloated derivative (dry state), 15 g.; ZnNO <sub>3</sub> ·6H <sub>2</sub> O, 2.25. Drying at 90° C. for 10 min. Condens. at 150° C. for 5 min. | 29.8/25.4 (55.2)            | 145/129 (274)  | 132/130 (262) | (1)                 | (1)    | 80.5                 | 20                              | -----  |
| 457..... | Methyloated derivative (dry state), 15 g.; CH <sub>3</sub> COOH, 6.65. Drying at 90° C. for 10 min. Condens. at 150° C. for 5 min.                 | 27.3/30.2 (57.5)            | 151/140 (291)  | 146/131 (277) | 5                   | 4.66   | 81                   | -3.25                           | 25.7   |

<sup>1</sup> Not evaluated.

is the angle obtained with the apparatus of the I.T.F. (Institute Textile de France), following the definition of the Societe pour la Diffusion d'Appareils de Mesures et de Controles.

The washings are carried out in an automatic washing machine of the domestic type, with a solution of 30 grams per litre of block soap in flakes and 15 grams per litre of anhydrous sodium carbonate per litre of tap-water. The operation is carried out up to boiling, the rinsing being effected up to the evacuation of all the alkaline water.

The evaluation of the wash and wear, that is to say the appearance of the fabric after washing, is carried out

45 is brought out clearly. The proportions of the catalyst were regulated in order that the deterioration of the fabric, shown by the fall in the dynamometric strength, is comparable in all the tests.

50 It can be seen that glyoxylic acid, while giving an excellent resistance to chlorine, also shows itself to be the best catalyst in respect of uncreasability.

#### EXAMPLE 2

The same procedure is followed as in Example 1, but with 25 grams per litre of methyloated product. The results are shown in Table II.

TABLE II

| Test No. | Bath formula and working conditions                                                                                                                                | Dynamo Strength (kg.) Wp/Wt | Uncreasability |               | W & W Monsanto test |        | Whiteness (as it is) | Scorch test A.A.T.C.C., percent |        |
|----------|--------------------------------------------------------------------------------------------------------------------------------------------------------------------|-----------------------------|----------------|---------------|---------------------|--------|----------------------|---------------------------------|--------|
|          |                                                                                                                                                                    |                             | As it is Wp/Wt | 2 wash Wp/Wt  | 2 wash              | 5 wash |                      | As it is                        | 5 wash |
| 357..... | Methyloated derivative (dry state), 25 g.; MgCl <sub>2</sub> ·3.75. Drying at 90° C. for 10 min. Condens. at 150° C. for 5 min.                                    | 28.3/26.2 (54.5)            | 132/137 (269)  | 141/137 (278) | 4.5                 | 5      | 81                   | 17.5                            | -----  |
| 303..... | Methyloated derivative (dry state), 25 g.; Zn(NO <sub>3</sub> ) <sub>2</sub> ·6H <sub>2</sub> O, 3.75. Drying at 90° C. for 10 min. Condens. at 150° C. for 5 min. | 30.6/32.4 (63)              | 135/135 (270)  | 118/118 (236) | (1)                 | (1)    | 81                   | 73                              | -----  |
| 306..... | Methyloated derivative (dry state), 25 g.; Zn(NO <sub>3</sub> ) <sub>2</sub> ·6H <sub>2</sub> O, 7.5. Drying at 90° C. for 10 min. Condens. at 150° C. for 5 min.  | 21.9/22.5 (44.4)            | 138/147 (285)  | 133/131 (264) | (1)                 | (1)    | 82.5                 | -7                              | -----  |
| 460..... | Methyloated derivative (dry state), 25 g.; CH <sub>3</sub> COOH, 11.25. Drying at 90° C. for 10 min. Condens. at 150° C. for 5 min.                                | 29.2/25.8 (55)              | 146/138 (284)  | 135/145 (280) | 5                   | 5      | 81                   | 3.28                            | 9.6    |

<sup>1</sup> Not evaluated.

**5**  
**EXAMPLE 3**

The same procedure is followed as for Example 1, but with 50 grams per litre of the methylolated product. The results are shown in Table III.

TABLE III

| Test No. | Bath formula and working conditions                                                                                                                                         | Dynamo Strength (kg.) Wp/Wt | Uncreasability   |                  | W & W Monsanto test |        | Whiteness (as it is) | Scorch test A.A.T.C.C., percent |        |
|----------|-----------------------------------------------------------------------------------------------------------------------------------------------------------------------------|-----------------------------|------------------|------------------|---------------------|--------|----------------------|---------------------------------|--------|
|          |                                                                                                                                                                             |                             | As it is Wp/Wt   | 2 wash Wp/Wt     | 2 wash              | 5 wash |                      | As it is                        | 5 wash |
| 378..... | Methylolated derivative (dry state), 50 g.;<br>MgCl <sub>2</sub> ·6H <sub>2</sub> O, 15.<br>Drying at 90° C. for 10 min.<br>Condens. at 150° C. for 5 min.                  | 22.4/20.1<br>(42.5)         | 144/147<br>(291) | 134/143<br>(277) | 4                   | 4.5    | 81                   | 67                              | -----  |
| 321..... | Methylolated derivative (dry state), 50 g.;<br>Zn(NO <sub>3</sub> ) <sub>2</sub> ·6H <sub>2</sub> O, 7.5.<br>Drying at 90° C. for 10 min.<br>Condens. at 150° C. for 5 min. | 23.4/21.1<br>(44.6)         | 148/149<br>(297) | 139/145<br>(284) | 4.25                | 4.35   | 79                   | 3                               | -----  |
| 463..... | Methylolated derivative (dry state), 50 g.;<br>CHOCOOH, 22.5<br>Drying at 90° C. for 10 min.<br>Condens. at 150° C. for 5 min.                                              | 22.9/20.5<br>(43.4)         | 152/154<br>(306) | 142/138<br>(280) | 5                   | 5      | 82.5                 | 6.65                            | 0      |

## EXAMPLE 4

The same procedure is followed as for Example 1, but with 75 grams per litre of methylolated product. The results are shown in Table IV.

TABLE IV

| Test No. | Bath formula and working conditions                                                                                                                                           | Dynamo Strength (kg.) Wp/Wt | Uncreasability   |                  | W & W Monsanto test |        | Whiteness (as it is) | Scorch test A.A.T.C.C., percent |        |
|----------|-------------------------------------------------------------------------------------------------------------------------------------------------------------------------------|-----------------------------|------------------|------------------|---------------------|--------|----------------------|---------------------------------|--------|
|          |                                                                                                                                                                               |                             | As it is Wp/Wt   | 2 wash Wp/Wt     | 2 wash              | 5 wash |                      | As it is                        | 5 wash |
| 384..... | Methylolated derivative (dry state), 75 g.;<br>MgCl <sub>2</sub> ·6H <sub>2</sub> O, 11.25.<br>Drying at 90° C. for 10 min.<br>Condens. at 150° C. for 5 min.                 | 21.9/19.2<br>(41.1)         | 146/149<br>(295) | 144/142<br>(286) | 5                   | 5      | 82                   | 32                              | -----  |
| 330..... | Methylolated derivative (dry state), 75 g.;<br>Zn(NO <sub>3</sub> ) <sub>2</sub> ·6H <sub>2</sub> O, 11.25.<br>Drying at 90° C. for 10 min.<br>Condens. at 150° C. for 5 min. | 20.7/18.5<br>(39.2)         | 150/146<br>(296) | 150/148<br>(298) | 5                   | 5      | 81                   | 0                               | -----  |
| 466..... | Methylolated derivative (dry state), 75 g.;<br>CHOCOOH, 33.75.<br>Drying at 90° C. for 10 min.<br>Condens. at 150° C. for 5 min.                                              | 23.8/22.9<br>(46.7)         | 160/155<br>(315) | 144/150<br>(294) | 5                   | 5      | 81.5                 | 4.1                             | 6.7    |

## EXAMPLE 5

As the impregnation solution, there was utilized a solution of 25 grams per litre of a cyclic urea-formol condensation product (prepared by condensing simultaneously 1 mol of glyoxal, 2 mols of formaldehyde and 1 mol of urea). The results are shown in Table V.

TABLE V

| Test No.  | Bath formula and working conditions                                                                                                                                           | Dynamo Strength (kg.) Wp/Wt | Uncreasability   |                  | W & W Monsanto test |        | Whiteness (as it is) | Scorch test A.A.T.C.C., percent |        |
|-----------|-------------------------------------------------------------------------------------------------------------------------------------------------------------------------------|-----------------------------|------------------|------------------|---------------------|--------|----------------------|---------------------------------|--------|
|           |                                                                                                                                                                               |                             | As it is Wp/Wt   | 2 wash Wp/Wt     | 2 wash              | 5 wash |                      | As it is                        | 5 wash |
| 411(a)... | Methylolated derivative (dry state), 25 g.;<br>Zn(NO <sub>3</sub> ) <sub>2</sub> ·6H <sub>2</sub> O, 7.5 g.<br>Drying at 90° C. for 10 min.<br>Condens. at 150° C. for 5 min. | 23.6/33.2<br>(46.8)         | 139/135<br>(274) | 133/139<br>(272) | 4                   | -----  | 80                   | 32                              | 74     |
| 536.....  | Methylolated derivative (dry state), 25 g.;<br>CHOCOOH, 12.5 g.<br>Drying at 90° C. for 10 min.<br>Condens. at 150° C. for 5 min.                                             | 25.5/24<br>(49.5)           | 136/135<br>(271) | 127/130<br>(257) | 4.75                | 4.5    | 82                   | -5.6                            | 4.1    |

## EXAMPLE 6

60

The same dressing solution was applied as in Example 5, but with a concentration of 75%. The results are shown in Table VI.

TABLE VI

| Test No. | Bath formula and working conditions                                                                                                                                            | Dynamo Strength (kg.) Wp/Wt | Uncreasability   |                  | W & W Monsanto test |        | Whiteness (as it is) | Scorch test A.A.T.C.C., percent |        |
|----------|--------------------------------------------------------------------------------------------------------------------------------------------------------------------------------|-----------------------------|------------------|------------------|---------------------|--------|----------------------|---------------------------------|--------|
|          |                                                                                                                                                                                |                             | As it is Wp/Wt   | 2 wash Wp/Wt     | 2 wash              | 5 wash |                      | As it is                        | 5 wash |
| 417..... | Methylolated derivative (dry state), 75 g.;<br>Zn(NO <sub>3</sub> ) <sub>2</sub> ·6H <sub>2</sub> O, 22.5 g.<br>Drying at 90° C. for 10 min.<br>Condens. at 150° C. for 5 min. | 18/15.3<br>(33.3)           | 146/149<br>(295) | 144/144<br>(288) | 4.5                 | -----  | 79                   | 7.2                             | 58     |
| 538..... | Methylolated derivative (dry state), 75 g.;<br>CHOCOOH, 37.5 g.<br>Drying at 90° C. for 10 min.<br>Condens. at 150° C. for 5 min.                                              | 19.9/18<br>(37.9)           | 139/147<br>(286) | 140/143<br>(292) | 4.75                | 4.75   | 82                   | 0                               | 0      |

7  
EXAMPLE 7

A solution of dimethylol glyoxal mono-ureine is employed at different concentrations. The results are given in Table VII.

| Test No. | Bath formula and working conditions                                                                       | Dynamo Strength (kg.)<br>Wp/Wt | Uncreasability    |                  | W & W Monsanto test |        | Whiteness (as it is) | Scorch test<br>A.A.T.C.C., percent |        |
|----------|-----------------------------------------------------------------------------------------------------------|--------------------------------|-------------------|------------------|---------------------|--------|----------------------|------------------------------------|--------|
|          |                                                                                                           |                                | As it is<br>Wp/Wt | 2 wash<br>Wp/Wt  | 2 wash              | 5 wash |                      | As it is                           | 5 wash |
| 548..... | Methylolated derivative (dry state), 25 g.; CHOCOOH, 12.5 g.<br>Drying for 10 min.<br>Condens. for 5 min. | 25.7/26.6<br>(52.3)            | 127/130<br>(257)  | 118/137<br>(255) | -----               | 4.25   | 83                   | 12.8                               | 21     |
| 550..... | Methylolated derivative (dry state), 75 g.; CHOCOOH, 37.5 g.<br>Drying for 10 min.<br>Condens. for 5 min. | 19.4/15.5<br>(34.9)            | 143/140<br>(283)  | 125/127<br>(252) | -----               | 4.75   | 82                   | 2.6                                | 17.6   |

## EXAMPLE 8

In this example, glyoxylic acid alone was employed as the anti-creasing agent. The results are shown in Table VIII.

impregnating bath consisting essentially of an aqueous solution of glyoxylic acid and at least one reactive dressing resin containing methylol groups and capable of reacting with the hydroxyl groups present in the cellulose

| Test No. | Bath formula and working conditions                                                                | Dynamo Strength (kg.)<br>Wp/Wt | Uncreasability    |                  | W & W Monsanto test |        | Whiteness (as it is) | Scorch test<br>A.A.T.C.C., percent |        |
|----------|----------------------------------------------------------------------------------------------------|--------------------------------|-------------------|------------------|---------------------|--------|----------------------|------------------------------------|--------|
|          |                                                                                                    |                                | As it is<br>Wp/Wt | 2 wash<br>Wp/Wt  | 2 wash              | 5 wash |                      | As it is                           | 5 wash |
| 501..... | 7.5 grams per litre of CHOCOOH.<br>Drying at 90° C. for 10 min.<br>Condens. at 150° C. for 5 min.  | 27/23.5<br>(50.5)              | 107/118<br>(225)  | 107/100<br>(207) | -----               | 4.5    | 82.5                 | +0.3                               | -7     |
| 502..... | 12.5 grams per litre of CHOCOOH.<br>Drying at 90° C. for 10 min.<br>Condens. at 150° C. for 5 min. | 25.1/24.1<br>(49.2)            | 121/125<br>(246)  | 100/112<br>(212) | -----               | 4.5    | 82.5                 | -2                                 | -5.2   |
| 504..... | 37.5 grams per litre of CHOCOOH.<br>Drying at 90° C. for 10 min.<br>Condens. at 150° C. for 5 min. | 19.4/19.5<br>(38.9)            | 130/148<br>(278)  | 114/117<br>(231) | -----               | 5      | 83                   | -2.1                               | -8.7   |

We claim:

1. A method of treatment of a fabric of cellulose fiber, comprising the steps of: immersing said fabric in an impregnating bath constituted by an aqueous solution comprising at least glyoxylic acid having a concentration of about 7.5 to 37.5 grams of glyoxylic acid per litre of said solution; squeezing out the aqueous solution in such manner that the increase in weight of such fabric is comprised between 2 to 20% and more; drying for about 10 minutes at about 90° C. and subjecting said fabric to a thermal operation for about 5 minutes at about 150° C.

2. A method of treatment of a fabric of cellulose fibre comprising the steps of: immersing said fabric in an impregnating bath consisting essentially of an aqueous solution of glyoxylic acid and at least one reactive dressing resin totally methylolated and capable of reacting with the hydroxyl groups present in the cellulose and selected from the group of the cyclic urea-formol resins, the proportion of glyoxylic acid with respect to said dressing being in a percentage from 10% to 100%; squeezing out the aqueous solution in such manner that the increase in weight of said fabric is comprised between 2 to 20% and more; drying and subjecting said fabric to a thermal operation.

3. A method of treatment of a fabric of cellulose fibre comprising the steps of: immersing said fabric in an impregnating bath consisting essentially of an aqueous solution of glyoxylic acid and at least one reactive dressing resin containing methylol groups and capable of reacting with the hydroxyl groups present in the cellulose and selected from the group of the cyclic urea-formol resins, the proportion of glyoxylic acid with respect to said dressing being in a percentage varying from 10% to 100%; squeezing out the aqueous solution in such manner that the increase in weight of said fabric is comprised between 5 and 12%; drying and subjecting said fabric to a thermal operation.

4. A method of treatment of a fabric of cellulose fibre, comprising the steps of: immersing said fabric in an

and selected from the group of the cyclic urea-formol resins, the proportion of glyoxylic acid with respect to said dressing being in a percentage comprised between 33 and 50%; squeezing out the aqueous solution in

such manner that the increase in weight of said fabric is comprised between 2 and 20% and more; drying and subjecting said fabric to a thermal operation.

5. A method of treatment of a fabric of cellulose fibre, comprising the steps of: immersing said fabric in an impregnating bath consisting essentially of an aqueous solution of glyoxylic acid and at least one reactive dressing resin containing methylol groups and capable of reacting with the hydroxyl groups present in the cellulose and selected from the group of the cyclic urea-formol resins, the proportion of glyoxylic acid with respect to said dressing being in a percentage varying from 33 to 50%; squeezing out the aqueous solution in such manner that the increase in weight of said fabric is comprised between 5 and 12%; drying and subjecting said fabric to a thermal operation.

6. A method of treatment of a fabric of cellulose fibre, comprising the steps of: immersing said fabric in an impregnating bath constituted by an aqueous solution comprising at least glyoxylic acid; squeezing out the aqueous solution in such manner that the increase in weight of said fabric is comprised between 2 and 20% and more; drying and subjecting said fabric to a thermal operation carried out at a temperature of 130° to 180° C. for a period of from one minute to one hour.

7. A method of treatment of a fabric of cellulose fibre, comprising the steps of: immersing said fabric in an impregnating bath constituted by an aqueous solution comprising at least glyoxylic acid; squeezing out the aqueous solution in such manner that the increase in weight of said fabric is comprised between 2 and 20% and more; drying and subjecting said fabric to a thermal operation carried out at 150° C. for 5 minutes.

8. A method of treatment of a fabric of cellulose fibre, comprising the steps of: immersing said fabric in an impregnating bath consisting essentially of an aqueous solution of glyoxylic acid and at least one reactive resin dressing containing methylol groups and capable of reacting with the hydroxyl groups present in the cellulose and selected from the group of the cyclic urea-

formol resins, the proportion of glyoxylic acid with respect to said resin dressing being in a percentage comprised between 10 and 100%; squeezing out the aqueous solution in such manner that the increase in weight of said fabric is comprised between 2 and 20% and more; drying and subjecting said fabric to a thermal operation carried out at a temperature of 130 to 180° C. for a period of from one minute to one hour.

9. A method of treatment of a fabric of cellulose fibre, comprising the steps of: immersing said fabric in an impregnating bath consisting essentially of an aqueous solution of glyoxylic acid and at least one reactive resin dressing containing methylol groups and capable of reacting with the hydroxyl groups present in the cellulose and selected from the group of the cyclic urea-formol resins, the proportion of glyoxylic acid with respect to said dressing being in a percentage comprised between 10 to 100%; squeezing out the aqueous solution in such manner that the increase in weight of the fabric is comprised between 5 and 12%; drying and subjecting said fabric to a thermal operation carried out at a temperature of 130 to 180° C. for a period of from one minute to one hour.

10. A method of treatment of a fabric of cellulose fibre, comprising the steps of: immersing said fabric in an impregnating bath consisting essentially of an aqueous solution of glyoxylic acid and at least one reactive resin dressing containing methylol groups and capable of reacting with the hydroxyl groups present in the cellulose and selected from the group of the cyclic urea-formol resins, the proportion of glyoxylic acid with respect to said dressing being in a percentage comprised

5

10

15

20

25

30

between 33 and 50%; squeezing out the aqueous solution in such manner that the increase in weight of the fabric is comprised between 2 and 20% and more; drying and subjecting said fabric to a thermal operation carried out at a temperature of 130 to 180° C. for a period of from one minute to one hour.

11. A method of treatment of a fabric of cellulose fibre, comprising the steps of: immersing said fabric in an impregnating bath consisting essentially of an aqueous solution of glyoxylic acid and at least one reactive resin dressing containing methylol groups and capable of reacting with the hydroxyl groups present in the cellulose and selected from the group of the cyclic urea-formol resins, the proportion of glyoxylic acid with respect to said dressing being in a percentage comprised between 33 and 50%; squeezing out the aqueous solution in such manner that the increase in weight of said fabric is comprised between 5 and 12%; drying and subjecting said fabric to a thermal operation carried out at a temperature of 130 to 180° C. for a period of from one minute to one hour.

#### References Cited

##### UNITED STATES PATENTS

2,898,238 8/1959 Van Loo et al.

NORMAN G. TORCHIN, *Primary Examiner*

J. P. BRAMMER, *Assistant Examiner*

U.S. Cl. X.R.

8—116, 116.2